

Feb. 3, 1925.

1,524,938

J. F. MAKOWSKI

PLASTER LATH

Filed Nov. 7, 1923



INVENTOR.

*John F. Makowski*  
BY *George J. Webster*  
ATTORNEY

Patented Feb. 3, 1925.

1,524,938

# UNITED STATES PATENT OFFICE.

JOHN F. MAKOWSKI, OF STOCKTON, CALIFORNIA, ASSIGNOR TO CALIFORNIA CEDAR PRODUCTS COMPANY, OF STOCKTON, CALIFORNIA.

## PLASTER LATH.

Application filed November 7, 1923. Serial No. 673,234.

*To all whom it may concern:*

Be it known that I, JOHN F. MAKOWSKI, a citizen of the United States, residing at Stockton, county of San Joaquin, State of California, have invented certain new and useful Improvements in Plaster Laths; and I do declare the following to be a full, clear, and exact description of the same, reference being had to the accompanying drawings, 10 and to the characters of reference marked thereon, which form a part of this application.

This invention relates to the building art and particularly to wall construction.

15 The object of the invention is to produce a plaster lath built upon a plaster board base of such strength as to best sustain the strains and stresses of the weight of the plaster and to form on the face of the plaster board a continuous mechanical key surface for adhering the plaster thereto. This type of plaster lath per se has been heretofore produced by me and the present invention relates specifically to the elementary construction or make-up of the lath and particularly the specific lamination or coating material used to adhere the mechanical key face to the plaster board base. After many 20 years of study and experiment and a trial 25 production in this art I have ascertained that to produce a commercially successful plaster board of this type it is essential that this lamination must be fire and moisture resistant to the highest possible degree and in addition thereto it must have very intense adhesive qualities in order to properly sustain the weight of the key surface 30 and plaster thereon.

35 Summing up therefore a successful lath 40 of this type must in its combination consist first of a strong nonpeeling plaster board for a base, and second must have its key surface strongly adhered to the base with a substantially fire and moisture proof lamination between the two. Failure to have 45 both of these essentials renders the product non-commercial.

I have therefore produced a lath made up 50 in detail as hereinafter set forth and 55 claimed, which detailed composition attains the objects of the invention.

The figure in the drawings is a cross sectional view of the plaster lath.

60 The base sheet or body of the lath is 65 preferably made up of what is known as

plaster board of that type in which plastic material 1 is introduced between two surface paper sheets 2 and 3 which, when the plastic material dries, is thoroughly adhered thereto. In using such a base for the support for the mechanical key or bond of the lath, the tenacity of this adhesive becomes a very decided factor in the production of a commercially successful lath. 60

Therefore the type of plaster board specifically shown and described in my co-pending application for patent, Serial No. 536,350, through the use of the adhesive dextrin as set forth therein, has provided the necessary tenacious adherence both for 70 the mass and the surface sheets so that "peelers" are eliminated and the plaster key or bond surface may be safely used thereon, as there is no danger of the weight of the plaster pulling the sheets loose or sagging 75 the board in any way.

Having found a suitable base for the lath my next problem was to provide the proper adhesive for cementing the mechanical key or bonding surface to the base support. 80 Fire underwriters' rules require that the lath meet their specifications and the trade demands that the lath, especially for exterior use, must be impervious to moisture. I have already made a great step in the direction of satisfying these demands by the production of a lath as set forth in my allowed case, Serial No. 608,595, in which I used casein as the essential adhesive ingredient. While this permits the production of a very fine grade of lath still, by experiment, I found the casein to be not as clearly water proof as I felt was necessary 85 to the greatest degree of perfection.

Further careful experimentation has 90 finally enabled me to determine that a cementitious composition made up of magnesite, with silicyl as a filler and magnesium chloride, to cause the composition to harden and set, substantially satisfies all requirements 95 as above enumerated.

The magnesite could be used alone without the body or carrier material but the latter is added in order to keep the cost 100 of the product as low as possible.

I use generally by bulk, one part magnesite, one and one half parts nineteen per cent (Baumé) solution of magnesium chloride and two parts diatomaceous earth.

105 This is applied to the surface of the 110

base board by suitable means and to a desired thickness to form a bed or coating 4. The finely divided mineral fragments 5 are then sprinkled into the wet mass by 5 suitable means. These mineral fragments become partially imbedded into the moist mass 4 and when the same hardens and sets they are permanently and inseparably cemented therein and to the base board. This 10 coating of the magnesite composition between the gravel and the base forms a substantially complete barrier to fire and moisture while at the same time furnishing the great adhesive qualities required.

15 When the magnesite composition is applied to the base board the chloride soaks into the paper surface and this tends to fire-proof the paper per se.

In the completed lath the wall board 20 forms the base or body thereof, the magnesite composition forms the water and fire proofing element and the adhesive in which is formed the mechanical key or bond, which latter in turn forms the key surface 25 to which the plaster is to be adhered.

From the foregoing description it will be readily seen that I have produced such a device as substantially fulfills the objects of the invention as set forth herein.

30 While this specification sets forth in detail the present and preferred construction of the device, still in practice such deviations from such detail may be resorted to as do not form a departure from the spirit 35 of the invention, as defined by the appended claims.

Having thus described my invention what I claim as new and useful and desire to secure by Letters Patent is:

40 1. A plaster lath comprising a base, a surface lamination of fire and water resist-

ing composition on the base, such composition consisting of magnesite and silicyl mixed with magnesium chloride; and a mechanical plaster key surface adhered to 45 the base through the medium of such composition.

2. A plaster lath comprising a plastic base having a paper sheet adhered thereto, and a mechanical plaster key adhered to 50 the sheet through the medium of a composition consisting essentially of magnesite and magnesium chloride.

3. A plaster lath comprising a base, a coating on the base in which magnesite 55 mixed with magnesium chloride is the essential element, and a plaster key adhered to such coating.

4. A plaster lath comprising a base, a composition coating having magnesite 60 mixed with magnesium chloride therein spread over the surface of the base, and a plaster key surface formed in the composition.

5. A plaster lath comprising a base, a 65 surface lamination of fire and water resisting composition on the base, such composition consisting of magnesite and diatomaceous earth mixed with magnesium chloride; and a mechanical plaster key surface 70 adhered to the base through the medium of such composition.

6. A plaster lath comprising a base, a composition coating having magnesite 75 mixed with magnesium chloride therein spread over the surface of the base, and a mechanical plaster key surface adhered to the base through the medium of said composition.

In testimony whereof I affix my signature.

JOHN F. MAKOWSKI.